

**1****3,732,128****HEAT TREATMENTS OF DIE CASTINGS  
UNDER PRESSURE**

Charles D. Statham, Trenton, N.J., assignor to N L  
Industries, Inc., New York, N.Y.  
No Drawing. Filed July 16, 1971, Ser. No. 163,480  
Int. Cl. C22f 1/04, 1/06

**U.S. Cl. 148—159****3 Claims****ABSTRACT OF THE DISCLOSURE**

Metallic die castings of magnesium, aluminum and alloys thereof are subjected to a heat treatment of from 300° to 600° C. under a pressure of from 100 to 10,000 p.s.i. followed by a low temperature aging treatment to improve the properties of the metals without forming blisters on the die cast product.

**BACKGROUND OF THE INVENTION**

High temperature heat treatments are usually not employed with die castings. Temperature treatments of 300 to 500° C. are sometimes used with sand and permanent mold castings or on wrought products. In these treatments, however, only atmospheric pressure is used. The treated metal or alloy is then usually subjected to a low temperature heat treatment of 100° C. to 250° C. to improve the properties of the metal or alloy.

Magnesium and aluminum metal and alloy die castings normally cannot be treated at temperatures of 300° C. to 500° C. without forming blisters on the surface of the metal or alloy.

**SUMMARY OF THE INVENTION**

A method for improving the mechanical properties of a metallic die casting selected from the group consisting of magnesium and aluminum and alloys thereof which comprises placing the die casting in a closed container, heating the die casting up to 300° C. to 600° C. under a pressure of from 100–10,000 p.s.i. for 1–72 hours and rapidly cooling said die casting while still maintaining the applied pressure. This heat treated die casting is then subjected to a low temperature aging treatment of from 100° C. to 250° C. for 1–72 hours at atmospheric pressure. These two heat treatments in combination improve the mechanical strength of die casting.

**DESCRIPTION OF THE PREFERRED  
EMBODIMENTS**

Both magnesium and aluminum metal and alloys thereof when subjected to a die casting operation form a die casting which is porous. This porous metal or alloy normally cannot be heated to a temperature of 300° C. to 600° C. because blisters form on the metallic surface. Blisters begin to form at about 300° C. for magnesium and about 350° C. for aluminum.

It has now been discovered that the porous die casting may be heated at 300° C. to 600° C. without forming blisters if pressure of 100–10,000 p.s.i. is employed during heat treatment.

**2**

This high temperature treatment followed by the low temperature heat treatment produces a die casting with increased mechanical strength properties which heretofore have not been obtained.

5 In order to describe the instant invention in more detail the following examples are presented:

**Example I**

In this example an aluminum alloy die casting weighing 10 200 gms. was placed in an autoclave. The die casting used was A.S.T.M.-SC84A. The die casting was heated to 480° C. at 2000 p.s.i. pressure for four hours.

After the heat treatment, the die casting was cooled rapidly and the pressure was released. This die casting was 15 then subjected to low temperature heat treatment of 175° C. for eight hours at atmospheric pressure.

The final die casting after high temperature heat treatment under pressure followed by the low temperature heat treatment was examined for its mechanical strength properties.

20 It was found that its yield strength was 50 k.s.i. compared to 25 k.s.i. for the untreated alloy die casting. This pressure treated die casting was substantially free from blisters due to the use of the pressure heat treatment.

**Example II**

In this run the procedure of Example I was repeated except that the aluminum alloy die casting used was A.S.T.M.-SN122A.

30 After the die casting was subjected to the pressure heat treatment followed by the low temperature treatment, the treated die casting was substantially free from blisters. The yield strength of the treated die casting was 60 k.s.i. compared with only 35 k.s.i. for the untreated die casting.

**Example III**

In this run a magnesium alloy die casting was used in place of an aluminum alloy. The magnesium alloy die casting was identified as A.S.T.M.-AZ91B. This particular die casting was pressure heat treated at 400° C. for 20 hours and rapidly cooled followed by the low temperature heat treatment at 175° C. for 24 hours at atmospheric pressure.

Again after subjecting the die casting to the high temperature and pressure heat treatment followed by the low temperature heat treatment, the final die casting had a 45 greater yield strength than the untreated die casting.

While this invention has been described and illustrated by the examples shown, it is not intended to be strictly limited thereto, and other variations and modifications 50 may be employed within the scope of the following claims:

What is claimed is:

1. A method for treating a metallic die casting selected 55 from the group consisting of a casting of aluminum, magnesium and an alloy thereof, to improve the mechanical properties of said die casting which comprises placing said die casting in a closed chamber, heating said casting at a temperature from 300° C. to 600° C. under a pressure of from 100 to 10,000 p.s.i. for a period from 1 to 72 hours and after said treatment, rapidly cooling said casting 60 while still under pressure, and then heating said casting of

**3**

a temperature of from 100° C. to 250° C. for 1 to 72 hours at atmospheric pressure and subsequently cooling said casting to room temperature.

2. Method according to claim 1 in which said die casting is an alloy of aluminum.

3. Method according to claim 1 in which said die casting is an alloy of magnesium.

**4**

|           |         |                     |           |
|-----------|---------|---------------------|-----------|
| 1,891,234 | 12/1932 | Langenberg -----    | 148—131 X |
| 3,156,974 | 11/1964 | Bobrowsky -----     | 148—4 X   |
| 3,157,540 | 11/1964 | Bobrowsky -----     | 148—131   |
| 3,329,535 | 7/1967  | Langer et al. ----- | 148—4     |

5

## OTHER REFERENCES

Alloy Digest, Filing Code Mg-36, Engr. Digest Inc., New Jersey, January 1958.

10 CHARLES N. LOVELL, Primary Examiner

U.S. CL. X.R.

UNITED STATES PATENTS

|           |        |              |         |
|-----------|--------|--------------|---------|
| 3,496,624 | 2/1970 | Kerr -----   | 148—4 X |
| 1,946,545 | 2/1934 | Pessel ----- | 148—131 |

148—131, 161

## References Cited